

## UNITED STATES PATENT OFFICE.

MORITZ FREIBERGER AND AUGUST HOLTmann, OF BERLIN-CHARLOTTENBURG,  
GERMANY.

## CALICO-PRINTING COLOR COMPOSITION AND PROCESS.

No Drawing. Application filed October 25, 1924, Serial No. 745,921, and in Germany December 14, 1923.

This invention comprises improvements in and connected with calico and like roller printing and the colors used therefor.

In the printing of calico by means of deeply engraved cylinders excess colors is removed by means of rollers or doctors and undesired markings frequently appear on the cylinders in a very objectionable manner. These markings become apparent by 10 the sudden appearance of smudges and streaks which extend right round the circumference of the cylinders and are reproduced in the print thereby spoiling the latter. The trouble aforesaid is still further increased by the necessity for stopping the 15 machine for the cleaning of the various cylinders and rollers and color containers or color boxes and sometimes it is even found to be necessary to renew the color supply. 20 The cause of these troubles, which have always been liable to occur, has heretofore been a matter of doubt. Apparently they are not due to a reaction of the printing color for they occur in the same manner with 25 acid printing color and with alkaline printing color such as the indanthrene printing colors. The fact that acid printing colors, and, to a greater extent, alkaline printing colors, injuriously affect the cylinders and rollers, is not of itself a sufficient explanation 30 of the sudden occurrence of the troubles referred to, which includes the markings aforesaid and the so-called copper-grinding or disintegration, for the same troubles are experienced with neutral printing colors 35 which are in common use.

It can be stated that the troubles referred to are not obviated by taking great care that the colors are free from insoluble and 40 hard particles. It has been thought by some that galvanic action or electric currents are responsible and by others it has been suggested that the color undergoes some change during printing owing to the heat, or increased concentration and so on, so that a crystalline separation occurs. However, no 45 proof is available as to the correctness of any one of these theories.

According to the improvements the troubles aforesaid are completely, or almost completely obviated by adding to the printing colors organic bodies insoluble in water or in the printing color and combining a very great molecular weight with a high degree

of viscosity suitable organic bodies for the purpose being further required to be liquid or soft at ordinary temperatures or at the temperature at which they are to be employed.

Examples of bodies suitable for use in accordance with these improvements are, the highest fractions of the distillation of mineral oils and residual tars which are liquid or soft. Further examples are the viscous fractions of the tar oils or the tars. Amongst suitable products of this nature may be mentioned vaseline for work at high temperatures, ceresine, and wet steam cylinder oils for work at low temperatures. In general the effect of these conditions can be increased if other bodies capable of raising the degree of viscosity are dissolved in the hydrocarbons or oil or tar constituents. Examples of these additional bodies are waxes, paraffins and like bodies of animal, vegetable or mineral origin. With printing colors in which starch is employed as a thickening medium, and particularly acid printing colors, it is found advantageous to dissolve or mix in or with the viscous substances to be added highly molecular fatty acids, as for example oleic acid, or castor oil fatty acid. These additions on the one hand, facilitate the even distribution in the printing color of the highly molecular substances and, on the other hand, serve for rendering the starch soluble during heating, such as is subsequently required for developing, fixing and finally treating the printing color.

It is known to add oil to the printing color for the formation of color lake in some cases and for increasing the smoothness of the printing color in other cases. In practice vegetable oils have been employed for this purpose but these, after a short time underwent a change during the printing process so that the desired effect was lost, and this occurred whether acid color or alkaline color was used. As contrasted with this practice, the additions in accordance with these present improvements consist of highly viscous highly molecular substances preferably belonging to the range of hydrocarbons and in any case having the capacity for remaining passive against the influence or action of the printing color.

Finally, it is suitable in some circumstances to add to the printing color, in ad-

dition to the substances embodied in accordance with these improvements, a medium capable of preventing frothing, thereby guaranteeing the homogeneity or uniformity 5 of the color introduced or applied to the printing elements. For example an addition of heavy benzine may be made for the purpose in known manner. By heavy benzine we mean petroleum and tar distillates 10 which are obtained between the range of 150-210° C.

Having now particularly described and ascertained the nature of our said invention, and in what manner the same is to be performed, we declare that what we claim is:

1. A cloth or calico printing composition which includes a water insoluble organic body of high molecular weight and of high viscosity.
2. A cloth or calico printing color including a highly viscous mineral hydrocarbon.
3. A cloth or calico printing body including a color body and a highly viscous mineral oil body.
4. A cloth or calico printing color including a viscous mineral oil.
5. A cloth or calico printing color in which starch is employed as a thickening medium which contains a viscous mineral 30 body and a fatty acid of the type of oleic acid and castor oil fatty acid.

6. A cloth or calico printing color in which starch is employed as a thickening medium which contains a viscous mineral oil and a fatty acid of the type of oleic 35 acid and castor oil fatty acid.

7. A printing composition for calico printing which includes a viscous body which is 40 passage against the influence of the printing color and a froth preventing agent.

8. A printing composition for calico printing which includes a viscous mineral oil and a heavy benzine.

9. A cloth or calico printing composition which includes a highly viscous mineral body 45 and a heavy benzine.

10. In the process of printing calico or cloth, the step which embraces the inking of the printing surfaces with a cloth or calico printing composition containing a viscous 50 emulsifiable mineral body.

11. In the process of printing calico or cloth, the step which embraces the inking of the printing surfaces with a cloth or calico printing composition containing an 55 emulsion of a high boiling mineral oil.

In testimony whereof we have affixed our signatures.

MORITZ FREIBERGER.  
AUGUST HOLTMANN.